# EUROPEAN PATENT SPECIFICATION

(11) **EP 2 011 918 B1**
(45) Date of publication and mention of the grant of the patent: **30.12.2009**
(21) Application number: 08290005.1
(22) Date of filing: 02.01.2008
(51) Int. Cl.: D06P 5/30, D06P 1/52, B41M 7/00

(54) **Printing method and printed matter**
Druckverfahren und gedruckter Artikel
Procédé d'impression et objet imprimé

(30) Priority: 02.07.2007 JP 2007173786
(43) Date of publication of application: 07.01.2009
(73) Proprietor: Mimaki Engineering Co., Ltd., Tomi-shi, Nagano 389-0512 (JP)
(72) Inventor: Souma, Seiichi, c/o Mimaki Engineering Co., Ltd., Tomi-city Nagano (JP); Ikeda, Kazuaki, c/o Mimaki Engineering Co., Ltd., Tomi-city Nagano (JP); Tabayashi, Isao, c/o Mimaki Engineering Co., Ltd., Tomi-city Nagano (JP)
(74) Representative: Uchida, Kenji

(56) References cited:
- EP-A- 1 234 910
- JP-A- 2005 246 734
- US-A- 5 962 149
- US-B1- 6 521 343

## Description

The present invention relates to a printing method, and a printed matter. More particularly, the present invention relates to a printing method, and a printed matter, for printing by inkjet system.

Conventionally, screen printing has been widely used for commercial printing. Generally used in screen printing is an ink containing a high-viscosity binder. In case of printing on a medium such as fabric, a printing providing fastness to washing can be conducted because of such ink.

Inventors of the present invention have studied about printing on a medium such as fabric by inkjet system. However, to improve the ink to be adapted to inkjet printing, lowering of viscosity is required. As the viscosity of ink is lowered, a problem such as poor fastness to washing arises.

Since the printing by inkjet system is a system in which ink is ejected out of micro holes, a workable ejected amount of ink leads to a poor volume of the binder on a surface of the medium such as fabric. Therefore, when a printed matter is washed in practical use, the printed surface may be rubbed physically. That is, the printed matter can not have sufficient fastness to washing and sufficient fastness to rubbing.

Conventionally, printing on a medium such as a fabric by inkjet system has been disclosed in various patent documents (for example, see JP-A-2-295787). However, in view of the problem about the fastness to washing and the fastness to rubbing as mentioned above, it is difficult to achieve suitable printing by these disclosed methods. In general, there is a trade-off relationship between improvement in fastness and operational reliability according to the increase in viscosity of ink in the inkjet system. It is technically difficult to obtain a printed matter (printed subject) which can satisfy commercial qualities only by ink. Therefore, it is an object of the present invention to provide a printing method, a printed matter, and a printer capable of solving the aforementioned problem.

Examples of coating compositions enabling ink-jet printing on a fabric medium are disclosed in documents EP 1 234 910, US 6 521 343 or US 5 962 142.

To solve the aforementioned problem, the present invention has the following arrangements.
(Arrangement 1) A printing method for printing on a washable fabric medium by inkjet system, comprises: a printing step for printing on the medium by the inkjet system using a water-based pigment ink containing an anionic resin; and a coating agent applying step for applying a water-based coating agent containing water-soluble cationic resin particles to the medium at least before or after the printing step. Fabric means, for example, a cloth formed in a plate shape made of fibers. The fabric may be a woven fabric, a knitted fabric (stockinette), a lace, a felt, or a non-woven fabric. Fibers composing the fabric may be cotton fibers or synthetic fibers.

Accordingly, for example, it is possible to print on a fabric medium (conduct water pigment printing) by the inkjet system while improving the fastness to washing and the fastness to rubbing. Therefore, it is possible to obtain an inkjet printed matter having excellent fastness to washing and excellent fastness to rubbing, for example. In addition, the fastness to washing and the fastness to rubbing are improved without spoiling the beauty of the appearance.

In the coating agent applying step, the water-based coating agent is applied by an applying system selected from a group consisting of, for example, an inkjet system, a splaying system, and a screen system. In the coating agent applying step, it is preferable to conduct heating and pressing after applying the water-based coating agent by the splaying system or the like. In this case, the fix level of the water-based coating agent relative to the water-based pigment ink is increased as compared to a case simply applying the water-based pigment ink and the water-based coating agent to be superposed on each other. In case of conducting the coating agent applying step after the printing step, the printed ink is preferably subjected to baking for drying the ink between the printing step and the coating agent applying step, for example. Therefore, the water-based coating agent is more suitably applied.

The pH of the water-based coating agent applied in the coating agent applying step is in a range of, for example, from 3 to 7. The viscosity of the water-based coating agent is in a range of, for example, from 1 to 250 mPa•s (at a temperature of 25°C). The resin solid content of the water-based coating agent after being applied is in a range of, for example, from 0.5 to 10 mg per a square centimeter at least in the printed portion on the medium.

(Arrangement 2) The water-based coating agent contains cationic polyurethane resin particles as the water-soluble cationic resin particles. Therefore, the fastness to washing is suitably improved while ensuring the flexibility. In addition, the adhesion and durability of the water-based coating agent are suitably improved.

The water-based coating agent contains the cationic polyurethane resin particles in an amount of, for example, from 1 to 50 % by mass, preferably from 2 to 25 % by mass, in solid content equivalent. The tensile force of the coating layer formed by the water-based coating agent is in a range of from 5 to 50MPa, preferably from 30 to 50 Mpa.

The resin skeleton of the cationic polyurethane resin particles is any one selected from a group consisting of polyester, polyether, and polycarbonate. It is especially preferable that the water-based coating agent contains, as the water-soluble cationic polyurethane resin particles, particles of a cationic polyurethane resin of polyether type having polyether resin skeleton. In this case, the water-based coating agent contains the cationic polyurethane resin particles of polyether type in an amount of from 5 to 50 % by mass in solid content equivalent.

(Arrangement 3) The water-based coating agent contains the cationic polyurethane resin particles in an amount of from 2 to 25 % by mass in solid content equivalent and further contains an antidrying agent in an amount of from 5 to 50 % by mass. Accordingly, nozzle clogging in an inkjet head can be suitably prevented, thereby also achieving further suitable printing by the inkjet system.

(Arrangement 4) A printed matter printed on a washable fabric medium by the inkjet system, comprises: the fabric medium; a printing layer which is formed by printing on the medium by the inkjet system using a water-based pigment ink containing an anionic resin; and a coating layer which is formed at least on and under the printing layer by applying a water-based coating agent containing water-soluble cationic resin particles. This arrangement obtains the same effects as the arrangement 1, for example.

According to the present invention, it is possible to suitably print on a fabric medium by inkjet system while improving the fastness to washing and the fastness to rubbing.

The above, and the other objects, features and advantages will be made apparent from the following description of the preferred embodiments, given as non-limiting examples, with reference to the accompanying drawings, in which:
Fig. 1 is an illustration showing a structural example of a printed matter 10 according to an embodiment of the present invention; and
Fig. 2 is a flow chart showing an example of a printing method for the printed matter 10;
wherein 10 ... printer, 12 ... medium, 14 ... printing layer, 16 ... coating layer.
Fig. 1 is an illustration showing a structural example of a printed matter 10 according to an embodiment of the present invention. The printed matter 10 is a printed matter (printed subject) printed by inkjet system and comprises a medium 12, a printing layer 14, and a coating layer 16.

The medium 12 is a medium which is washable fabric. This fabric may be a woven fabric, a knitted fabric (stockinette), a lace, a felt, or a non-woven fabric. Fibers composing the fabric may be cotton fibers or synthetic fibers.

The printing layer 14 is a layer of ink printed on the medium 12 by the inkjet system. In this embodiment, the printing layer 14 is formed by water-based pigment ink containing an anionic resin. The coating layer 16 is a layer formed by applying a water-based coating agent containing water-soluble cationic resin particles. In this embodiment, the coating layer 16 is formed on the printing layer 14. According to this structure, the surface of the printing layer 14 is covered, thereby suitably improving the fastness to washing and the fastness to rubbing.

The coating layer 16 may be formed under the printing layer 14. According to this structure, for example, the adhesion between the printing layer 14 and the medium 12 is increased, thereby suitably improving the fastness to washing and the fastness to rubbing. The coating layers 16 may be formed both on and under the printing layer 14.

Fig. 2 is a flow chart showing an example of a printing method for the printed matter 10. The printing method is a method for printing on a medium 12, which is washable fabric, by the inkjet system. In the printing method, first, the medium 12 is prepared by, for example, mounting the fabric medium 12 to a printer (preparing step S 102).

Then, printing is carried out on the medium 12 by the inkjet system using the water-based pigment ink containing an anionic resin (printing step S104). After that, the water-based coating agent containing water-soluble cationic resin particles is applied to the medium 12 (coating agent applying step S106).

In this manner, it is possible to print on the fabric medium 12 (conduct water pigment printing) by the inkjet system while improving the fastness to washing and the fastness to rubbing. In addition, the fastness to washing and the fastness to rubbing are improved without spoiling the beauty of the appearance. Therefore, according to this embodiment, it is possible to obtain an inkjet printed matter having excellent fastness to washing and excellent fastness to rubbing, for example. It should be noted that, in case of forming the coating layer 16 under the printing layer 14, the water-based coating agent is applied to the medium 12 before the printing step S104.

In the coating agent applying step S106, the coating agent is applied by an applying system selected from a group consisting of, for example, an inkjet system, a splaying system, and a screen system. In the coating agent applying step S 106, it is preferable to conduct heating and pressing after applying the water-based coating agent by the splaying system or the like. In this case, the fix level of the water-based coating agent relative to the water-based pigment ink is increased.

The pH of the water-based coating agent applied in the coating agent applying step S106 is in a range of, for example, from 3 to 7. The viscosity of the water-based coating agent is in a range of, for example, from 1 to 250 mPa•s (at a temperature of 25°C). The resin solid content of the water-based coating agent after being applied is in a range of, for example, from 0.5 to 10 mg per a square centimeter at least in the printed portion on the medium.

The water-based coating agent contains cationic polyurethane resin particles as the water-soluble cationic resin particles. In this case, the fastness to washing is suitably improved while ensuring the flexibility.

The water-based coating agent contains the cationic polyurethane resin particles in an amount of, for example, from 1 to 50 % by mass, preferably from 2 to 25 % by mass, in solid content equivalent. The tensile force of the coating layer formed by the water-based coating agent is in a range of from 5 to 50MPa, preferably from 30 to 50 Mpa.

The resin skeleton of the cationic polyurethane resin particles is any one selected from a group consisting of polyester, polyether, and polycarbonate. It is especially preferable that the water-based coating agent contains, as the water-soluble cationic polyurethane resin particles, particles of a cationic polyurethane resin of polyether type having polyether resin skeleton.

The water-based coating agent contains the cationic polyurethane resin particles in an amount of from 2 to 25 % by mass in solid content equivalent and further contains an antidrying agent in an amount of from 5 to 50 % by mass. Accordingly, nozzle clogging in an inkjet head can be suitably prevented, thereby also achieving further suitable printing by the inkjet system.

Hereinafter, the present invention will be described in further detail with reference to Examples and Comparative Examples. Since conditions as will be described below are for Examples, the present invention is not limited thereto. For example, the amount of the water-soluble cationic resin particles (cationic polyether-urethane resin particles) in the water-based coating agent and the applying amount can be changed depending on the surface roughness and thickness of the printed matter, and target texture.

### (Example 1)

As the water-based coating agent of Example 1, an overcoating agent of a composition (Composition A) containing 50% Hydran CP-7030 available from Dainippon Ink and Chemicals Incorporated and 50% water was used. Hydran CP7030 contains 22% resin content of polyester resin. In Example 1, after printing with color inks, the water-based coating agent of the aforementioned composition A was applied. The amount of resin solid content in the coating agent after being applied was 1.1 mg per a square centimeter.

### (Example 2)

As the water-based coating agent of Example 2, an overcoating agent of a composition (Composition B) containing 50% Hydran CP-7020 available from Dainippon Ink and Chemicals Incorporated and 50% water was used. Hydran CP7020 contains 40% resin content of polycarbonate resin. In Example 2, after printing with color inks, the water-based coating agent of the aforementioned composition B was applied. The amount of resin solid content in the coating agent after being applied was 1.9 mg per a square centimeter.

### (Comparative Example 1)

In Comparative Example 1, only printing with color inks was conducted, that is, application of water-based coating agent was not conducted.

### (Evaluation)

Test for effect of improving the fastness to washing and the fastness to rubbing was carried out by the following procedure.
(1) In the printing step, a pattern of A4 size (624 square centimeter) is printed on a T shirt as the fabric medium with an inkjet printing pigment as the water-based pigment ink containing an anionic resin.
(2) The printed pattern is subjected to baking at a temperature 160°C for 60 seconds.
(3) In the coating agent applying step, 6g of the overcoating agent is applied to the printed pattern by a hand spray. After the application, the coating agent applied portion is subjected to curing by hot press.
(4) Testing of the fastness to washing and the fastness to rubbing is carried out according to JIS dyeing inspection.

Used as the color ink for printing was a printing pigment (color: cyan) manufactured by Mimaki Engineering Co., Ltd. The printing was conducted under conditions of 720-720 dpi, one-way printing, 2-pass 1-coat, and 100% print density.

Used as the T shirt was a white T shirt. The curing conditions for the overcoating agent were 160°C and 180 sec. The tests for the fastness to washing and the fastness to rubbing were carried out with Tokyo office of Japan Dyers' Inspection Institute Foundation as an inspection agency.

Table 1 shows results of the tests of the fastness to washing and the fastness to rubbing. The fastness to washing was fastness to washing according to JIS L 0844 A-2. The fastness to rubbing was fastness to rubbing according to JIS L 0849II.

**[Table 1]**

| | Fastness to washing [discoloration] | Fastness to rubbing [dry condition] | Fastness to rubbing [wet condition] |
|---|---|---|---|
| Example 1 | 5 | 4 | 3 |
| Example 2 | 4-5 | 3 | 3 |
| Comparative Example 1 | 4 | 2 | 2 |

As shown in Table, it was found that the fastness to washing of each of Examples 1 and 2 was improved as compared to Comparative Example 1. It was also found that the fastness to rubbing of each of Examples 1 and 2 was improved both in cases of the dry condition and the wet condition as compared to Comparative Example 1.

## Claims

1. A printing method for printing on a washable fabric medium (12) by inkjet system, comprising:
a printing step (104) for printing a printing layer (14) on the medium (12) by the inkjet system using a water-based pigment ink containing an anionic resin; and
a coating agent applying step (106) for applying a water-based coating agent containing water-soluble cationic resin particles to the medium at least after the printing step.

2. A printing method according to claim 1, comprising:
a coating agent applying step for applying said water-based coating agent to the medium before the printing step, such that a coating layer (16) is formed both on and under the printing layer (14).

3. A printing method according to claim 1 or 2, wherein said water-based coating agent contains cationic polyurethane resin particles as said water-soluble cationic resin particles.

4. A printing method as claimed in claim 3, wherein said water-based coating agent contains said cationic polyurethane resin particles in an amount of from 2 to 25 % by mass in solid content equivalent and further contains an antidrying agent in an amount of from 5 to 50 % by mass.

5. A printed matter printed by an inkjet system, said printer matter comprising:
a washable fabric medium (12) ;
a printing layer (14) formed by printing on said medium by the inkjet system using a water-based pigment ink containing an anionic resin;
said printer matter being **characterized in that** it comprises a first coating layer (16) formed at least on said printing layer (14) by applying a water-based coating agent containing water-soluble cationic resin particles.

6. A printed matter according to claim 5, **characterized in that** it comprises a second coating layer (16) formed under said printing layer (14) by applying a water-based coating agent containing water-soluble cationic resin particles.

## Patentansprüche

1. Druckverfahren zum Bedrucken eines waschbaren Textilmediums (12) durch ein Tintenstrahlsystem, umfassend:
eine Druckstufe (104) zum Bedrucken des Mediums (12) mit einer Druckschicht (14) durch das Tintenstrahlsystem unter Verwendung einer Pigmenttinte auf Wasserbasis mit einem Gehalt an einem anionischen Harz; und
eine Beschichtungsmittel-Auftragestufe (106) zum Auftragen eines Beschichtungsmittels auf Wasserbasis mit einem Gehalt an wasserlöslichen kationischen Harzteilchen auf das Medium zumindest nach der Druckstufe.

2. Druckverfahren nach Anspruch 1, umfassend:
eine Beschichtungsmittel-Auftragestufe zum Auftragen des Beschichtungsmittels auf Wasserbasis auf das Medium vor der Druckstufe, so dass eine Überzugsschicht (16) sowohl auf als auch unter der Druckschicht (14) gebildet wird.

3. Druckverfahren nach Anspruch 1 oder 2, wobei das Beschichtungsmittel auf Wasserbasis kationische Polyurethanharzteilchen als wasserlösliche kationische Harzteilchen enthält.

4. Druckverfahren nach Anspruch 3, wobei das Beschichtungsmittel auf Wasserbasis die kationischen Polyurethanharzteilchen in einer Menge von 2 bis 25 Masse-% im Feststoffanteil-Äquivalent enthält und ferner ein Antitrocknungsmittel in einer Menge von 5 bis 50 Masse-% enthält.

5. Durch ein Tintenstrahlsystem bedruckter Gegenstand, wobei der bedruckte Gegenstand folgendes umfasst:
ein waschbares Textilmedium (12);
eine Druckschicht (14), die durch Bedrucken des Mediums durch ein Tintenstrahlsystem unter Verwendung einer Pigmenttinte auf Wasserbasis mit einem Gehalt an einem anionischen Harz gebildet worden ist;
wobei der bedruckte Gegenstand **dadurch gekennzeichnet ist, dass** er eine erste Überzugsschicht (16) umfasst, die zumindest auf der Druckschicht (14) durch Auftragen eines Beschichtungsmittels auf Wasserbasis mit einem Gehalt an wasserlöslichen kationischen Harzteilchen gebildet worden ist.

6. Bedruckter Gegenstand nach Anspruch 5, **dadurch gekennzeichnet, dass** er eine zweite Überzugsschicht (16) umfasst, die unter der Druckschicht (14) durch Auftragen eines Beschichtungsmittels auf Wasserbasis mit einem Gehalt an wasserlöslichen kationischen Harzteilchen gebildet worden ist.

## Revendications

1. Procédé d'impression destiné à imprimer sur un support en tissu lavable (12) par un dispositif à jet d'encre, comprenant :
une étape d'impression (104) destinée à imprimer une couche d'impression (14) sur le support (12) par le dispositif à jet d'encre en utilisant une encre à pigment à base aqueuse contenant une résine anionique ; et
une étape d'application d'agent de revêtement (106) destinée à appliquer un agent de revêtement à base aqueuse contenant des particules d'une résine cationique soluble dans l'eau sur le support, au moins après l'étape d'impression.

2. Procédé d'impression selon la revendication 1, comprenant :
une étape d'application d'agent de revêtement destinée à appliquer ledit agent de revêtement à base aqueuse sur le support avant l'étape d'impression, de telle sorte qu'une couche de revêtement (16) est formée à la fois au-dessus et au-dessous de la couche d'impression (14).

3. Procédé d'impression selon la revendication 1 ou 2, dans lequel ledit agent de revêtement à base aqueuse contient des particules de résine de polyuréthanne cationique en tant que lesdites particules de résine cationique soluble dans l'eau.

4. Procédé d'impression selon la revendication 3, dans lequel ledit agent de revêtement à base aqueuse contient lesdites particules de résine de polyuréthanne cationique en une quantité de 2 à 25 % en masse de teneur solide équivalente et contient, en outre, un agent anti-séchage en une quantité de 5 à 50 % en masse.

5. Matière imprimée, imprimée par un dispositif à jet d'encre, ladite matière imprimée comprenant :
un support en tissu lavable (12) ;
une couche d'impression (14) formée par impression sur ledit support par le dispositif à jet d'encre en utilisant une encre à pigment à base aqueuse contenant une résine anionique ;
ladite matière imprimée étant **caractérisée en ce qu'**elle comprend une première couche de revêtement (16) formée au moins sur ladite couche d'impression (14) par application d'un agent de revêtement à base aqueuse contenant des particules d'une résine cationique soluble dans l'eau.

6. Matière imprimée selon la revendication 5, **caractérisée en ce qu'**elle comprend une seconde couche de revêtement (16) formée au-dessous de ladite couche d'impression (14) par application d'un agent de revêtement à base aqueuse contenant des particules de résine cationique soluble dans l'eau.
